# EUROPEAN PATENT APPLICATION

(11) **EP 0 384 411 A1**
(43) Date of publication of application: **29.08.1990**
(21) Application number: 90103268.0
(22) Date of filing: 20.02.1990
(51) Int. Cl.: G03C 1/73, G03C 7/00, B41M 5/26, B41M 5/34

(54) **Photochromic recording medium**

(30) Priority: 22.02.1989 JP 42607/89; 28.04.1989 JP 110454/89
(71) Applicant: SEIKO INSTRUMENTS INC., Tokyo 136 (JP)
(72) Inventor: Takahashi, Hiroshi, c/o Seiko Instruments Inc., Koto-ku, Tokyo (JP); Iwasaki, Fumiharu, c/o Seiko Instruments Inc., Koto-ku, Tokyo (JP); Sakojiri, Hiromichi, c/o Seiko Instruments Inc., Koto-ku, Tokyo (JP)
(74) Representative: Fleuchaus, Leo, Dipl.-Ing.

(57) **Abstract**

A photochromic recording paper. Photochromic material composed of triphenylmethane compound is impregnated in a paper substrate and is responsive to irradiation of optical ray effective to develop the photochromic material so as to effect recording of image on the substrate, the triphenylmethane compound having general composition represented by the following formula:

## Description

### BACKGROUND OF THE INVENTION

The present invention relates monocolor or multicolor photochromic recording paper of the type effective to record monocolor or multicolor continuously gradated image of high resolution and high quality, and of the type being easily produced and having simplified layer structure.

The conventional information recording papers include thermal recording papers of the thermo-sensitive type and electric-current-activated thermo-sensitive type, and include photo-recording paper of the diazo type, and other types utilizing silver salts or photochromic material. Particularly, the recording paper of the type utilizing photochromic compound is disclosed in, for example, Japanese laid-open patent application No 21128/1972, in which a substrate is coated thereon with a photochromic photo-sensitive layer which contains organic photochromic compound such as spiro compound so as to form double layer structure. Further, the Japanese laid-open patent application No. 147735/1983 discloses a recording medium of the type having a photo-sensitive substance layer containing two different compounds of an activator in the form of poly-halogen compound and a color former in the form of diphenylmethane compound.

However, the conventional recording paper has the following drawbacks.

With regard to the conventional thermal recording paper, there are drawbacks that only two-level recording is carried out and therefore continuously gradated image of high quality is not obtained. Further, there is another drawback that high resolution image cannot be obtained because of dependency of the image resolution on the dimension of a recording head heating element. Further, since the thermal multicolor recording is carried out according to application of thermal energy, the continuous gradation image cannot be obtained. Moreover, one color tone related to relatively low thermal energy is subsidiarily developed along edge of the image of another color tone related to relatively high thermal energy due to heat diffusion, thereby causing color dislocation.

With regard to the conventional photo-recording paper, the diazo photo-sensitive paper requires development process after exposure process. This process is of wet type. Further, since developer liquid is composed of ammonia-containing solution, there is caused a problem of bad smell.

With regard to the silver salt photography, there is a serious drawback that the silver salt of photo-sensitive substance must have uniform particle size and must be finely pulverized according to high technology and complicated process. Further, there are other drawbacks that exposure and development requires complicated process steps in wet manner. Moreover, in order to obtain multicolor image, it is necessary to superpose thin films in multi-layer structure including a photo-sensitive layer, transient layer, separating layer and filter layer for each of the three primary color tones, thereby causing a problem such as complicated manufacturing process.

With regard to the recording paper of the type utilizing photochromic compound, for example, in the Japanese laid-open patent application No. 21128/1972, the recording paper has a multi-layer structure in which a photochromic photo-sensitive layer containing organic photochromic compound and a separative undercoat layer are disposed on a substrate, thereby causing a problem that the manufacturing thereof needs complicated process. In the other Japanese laid-open patent application No 147735/1983, two different compounds of an activator and a developer are contained in a photo-sensitive substance layer and the photo-sensitive substance layer is disposed on a substrate to form a double-layer structure, thereby causing a problem that complicated steps are needed to produce the recording paper. Further, there is another problem of need for a plurality of printing steps including thermal process step.

### SUMMARY OF THE INVENTION

In view of the above noted problems of the prior art, an object of the present invention is to provide monocolor or multicolor photochromic recording paper responsive to irradiation of optical ray to record monocolor or multicolor continuously gradated image of high resolution and high quality, and of the type not having a complicated multi-layer structure and produced by simplified manufacturing processes.

According to the present invention, in order to achieve the above noted object, the inventive recording medium has structure in which at least one kind of triphenylmethane compound is impregnated in a substrate as photo-sensitive color former.

The inventive monocolor or multicolor photochromic recording paper is irradiated with optical ray to develop the photo-sensitive color former to record monocolor or multicolor image of high resolution. Further, by changing intensity of irradiating optical ray or exposure time interval thereof, monocolor or multicolor continuously gradated image can be recorded with high quality. In addition, by utilizing different photo-sensitive color formers having different activating wavelength, the photo-sensitive layer can be selectively developed according to wavelength of the irradiating optical ray to thereby record multicolor image. Moreover, since the photo-sensitive color former is directly impregnated in the substrate, hence the single layer structure is realized without complicated layer structure and the simplicated method of production is realized.

According to the present invention, the monocolor or multicolor photochromic recording medium is characterized in that at least one kind of triphenylmethane compound is impregnated in the substrate as the photo-sensitive color former which is responsive to optical ray irradiated onto the substrate to activate the photo-sensitive color former to record monocolor or multicolor image. The triphenylmethane compound is represented by the following formula: where X₁, X₂ and X₃ denote: hydrogen atom, halogen atom, alkyl group, alkoxyl group, amino group including the type in which hydrogen atom is substituted by alkyl group, alkoxyl group, alkyl halide group, phenyl group or phenyl halide group, and nitro group,
Y₁ and Y₂ denote: hydrogen atom, halogen atom, alkyl group, alkoxyl group, and amino group including the type in which hydrogen atom is substituted by alkyl group, alkoxyl group, alkyl halide group, phenyl group or phenyl halide group,
and Z denotes: hydroxyl group, cyano group, alkoxyl group and halogen atom.

Generally, photochromic compound is known as the substance exhibits color change due to incident light. Such compounds include spiropyran compound, fulgide compound, aniline compound, azobenzene compound, benzyl-pyridine compound, and tetrachlorodihydronaphthalene compound, etc. The spiropyran compound includes the followings:
1,3,3-trimethylindolyno-6′-nitro-2,2′-benzopyrylspirane, and 1,3,3-trimethylindolyno-8′-carboxybenzopyrylspirane.
The fulgide compound includes the followings:
(E)-α-3-furylethylidene(isopropylidene)succinic acid anhydride, (E)-α-(2,5-dimethyl-3-furylethylidene (isopropylidene)succinic acid anhydride, and (E)-2-[α-(2,5-dimethyl-3-thienyl)ethylidene]-3-isopropylidene succinic acid anhydride.
The aniline compound includes the followings:
Salicyliden aniline, salicyliden-m-toluidine, and salicyliden-p-phenetidine.
The azobenzene compound includes the followings:
azobenzene, p-dimethylaminoazobenzene, and p-dimethylaminoazobenzene-o-carbonate.
The benzylpyridine compound includes the followings:
benzylpyridine, and dinitrobenzylpyridine.
The tetrachlorodihydronaphthalene compound includes the followings:
tetrachloro-α-diketo-dihydronaphthalene, and tetra-chloro-1-keto-dihydronaphthalene.

However, these compounds exhibit photochromism only in a solution or in a polymer matrix. Therefore, in application to the recording medium, these photochromic compounds are conventionally dispersed in a polymer matrix layer which is disposed on a substrate.

On the other hand, according to the present invention, the triphenylmethane compound is utilized as photo-sensitive color former exhibiting photochromism. At least one kind of the triphenylmethane compound is directly applied to the substrate, such that the photo-sensitive color former is developed upon irradiation of optical ray. Further, each different triphenylmethane compound is selectively developed according to wavelength of the irradiating optical ray to record multicolor image.

The triphenyl compound used in the present invention is dissociated to a triphenylmethyl cation and another anion by the irradiation of optical ray to form color to thereby effect recording without additional development process as shown by the following relation (1):

### BRIEF DESCRIPTION OF THE DRAWINGS

Fig. 1 is a diagram showing light absorption spectrum of the inventive photochromic recording paper utilizing malachite green leuco cyanide; Fig. 2 is a diagram showing the relation between the irradiation time of optical ray and the color density of the photochromic recording paper utilizing malachite green leuco cyanide; Fig. 3 is a diagram showing light absorption spectrum of the inventive photochromic recording paper utilizing brilliant green leuco cyanide; Fig. 4 is a diagram showing the relation between the irradiation time of optical ray and the color density of the photochromic recording paper utilizing brilliant green leuco cyanide; Fig. 5 is a diagram showing light absorption spectrum of the inventive photochromic recording paper utilizing crystal violet leuco cyanide; Fig. 6 is a diagram showing the relation between the irradiation time of optical ray and the color density of the photochromic recording paper utilizing crystal violet leuco cyanide; Fig. 7 is a diagram showing light absorption spectrum of the inventive photochromic recording paper utilizing rosaniline leuco cyanide; Fig. 8 is a diagram showing the relation between the irradiation time of optical ray and the color density of the photochromic recording paper utilizing rosaniline leuco cyanide; Fig. 9 is a diagram showing light absorption spectrum of the inventive photochromic recording paper utilizing pararosaniline leuco cyanide; Fig. 10 is a diagram showing the relation between the irradiation time of optical ray and the color density of the photochromic recording paper utilizing pararosaniline leuco cyanide; Fig. 11 is a diagram showing light absorption spectrum of the inventive multicolor photochromic recording paper utilizing malachite green leuco cyanide and rosaniline leuco cyanide, where the solid line 1 denotes the light absorption spectrum after irradiation of 340 nm optical ray and the broken line 2 denotes the light absorption spectrum after irradiation o£ 300 nm optical ray; Fig. 12 is a diagram showing the relation between the irradiating time interval and the color density of the inventive multicolor photochromic recording paper utilizing malachite green leuco cyanide and rosaniline leuco cyanide, where the curve 3 indicates the relation when the 340 nm optical ray is irradiated, and the other curve 4 denotes the relation when the 300 nm optical ray is irradiated; Fig. 13 is a diagram showing light absorption spectrum of the inventive multicolor photochromic recording paper utilizing malachite green leuco cyanide and pararosaniline leuco cyanide, where the solid line 5 denotes the light absorption spectrum after irradiation of 340 nm optical ray and the broken line 6 denotes the light absorption spectrum after irradiation of 300 nm optical ray; Fig. 14 is a diagram showing the relation between the irradiating time interval and the color density of the inventive multicolor photochromic recording paper utilizing malachite green leuco cyanide and pararosaniline leuco cyanide, where the curve 7 indicates the relation when the 340 nm optical ray is irradiated, and the other curve 8 denotes the relation when the 300 nm optical ray is irradiated; Fig. 15 is a diagram showing light absorption spectrum of the inventive multicolor photochromic recording paper utilizing brilliant green leuco cyanide and rosaniline leuco cyanide, where the solid line 9 denotes the light absorption spectrum after irradiation of 340 nm optical ray and the broken line 10 denotes the light absorption spectrum after irradiation of 300 nm optical ray; Fig. 16 is a diagram showing the relation between the irradiating time interval and the color density of the inventive multicolor photochromic recording paper utilizing brilliant green leuco cyanide and rosaniline leuco cyanide, where the curve 11 indicates the relation when the 340 nm optical ray is irradiated, and the other curve 12 denotes the relation when the 300 nm optical ray is irradiated; Fig. 17 is a diagram showing light absorption spectrum of the inventive multicolor photochromic recording paper utilizing brilliant green leuco cyanide and pararosaniline leuco cyanide, where the solid line 13 denotes the light absorption spectrum after irradiation of 340 nm optical ray and the broken line 14 denotes the light absorption spectrum after irradiation of 300 nm optical ray; and Fig. 18 is a diagram showing the relation between the irradiating time interval and the color density of the inventive multicolor photochromic recording paper utilizing brilliant green leuco cyanide and pararosaniline leuco cyanide, where the curve 15 indicates the relation when the 340 nm optical ray is irradiated, and the other curve 16 denotes the relation when the 300 nm optical ray is irradiated.

### DETAILED DESCRIPTION OF THE INVENTION

For one embodiment of the present invention, the description is given for the monocolor photochromic recording paper in which the single photo-sensitive color former is comprised of a particular triphenylmethane compound, i.e., malachite green leuco cyanide represented by the following structural formula: This compound is dissolved in a solvent (chloroform). The solution is impregnated in a plain paper substrate and dried to form the recording paper. This photochromic recording paper forms green color by the irradiation of optical ray. Fig. 1 shows light absorption spectrum of the thus developed photochromic recording paper. As shown in the figure, the light absorption spectrum after the irradiation indicates the forming of green color as represented by the solid line thereby recognizing color change, while the light absorption spectrum before the irradiation indicates white color tone.

Further, as shown in Fig. 2, the color density is changed by controlling the irradiating time interval of the optical ray. For example, when the irradiating time interval is 1 sec, the color density is 0.095. When the irradiating time interval is 2 sec, the color density is 0.385. Consequently, the color density can be controlled according to the irradiating time interval.

For another embodiment of the present invention, the description is given for a multicolor photochromic recording paper constructed such that two particular triphenylmethane compounds are selected as the photo-sensitive color former, and the two compounds are dissolved into solvent (acetone) and then applied to a plain paper substrate and dried. The two particular compounds are malachite green leuco cyanide and rosaniline leuco cyanide as represented by the following composition formulas:

This multicolor photochromic recording paper forms green color due to development of malachite green leuco cyanide in response to 340 nm of wavelength of irradiating optical ray, and forms dark blue color which is mixture of green color due to development of malachite green leuco cyanide and magenta color due to development of rosaniline leuco cyanide in response to 300 nm of wavelength of irradiating optical ray.

Fig. 11 shows a light absorption spectrum of the thus developed multicolor photochromic recording paper, and Fig. 12 shows the relation between the irradiating time interval and the color density of the developed multicolor photochromic recording paper (hereinafter, the color density is determined by relative intensity with respect to each of the three primary filters). As shown in Fig. 11, while light absorption spectrum indicates white color before the irradiation optical ray, the light absorption spectrum after the irradiation of 340 optical ray indicates forming of green color as shown by solid line 1, and the other light absorption spectrum after the irradiation of 300 nm optical ray indicates forming of dark blue color as shown by the broken line 2, thereby realizing the color change.

This color forming can be explained according to the following relations (2): Namely, in the structure (a) or (c) before the color forming, the central carbon atom is bonded according to sp³ hybridized orbital. Upon irradiation of optical ray, ion dissociation is induced as shown by the structure (b) or (d) so that the central carbon atom is shifted to another bonding state according to sp² hybridized orbital. Consequently, in the structure (b) or (d), the conjugate bonding effect is extended throughout the molecule to thereby absorb visible light to cause color forming. This photo-ion-dissociation reaction has different activating wavelength due to difference of electron energy level and coupling dissociation energy of specific triphenylmethane compound depending on kinds of substitution group (indicated by X₁ through X₃, and Y₁ through Y₃ of the general formula) bonded to each phenyl group and depending on kinds of the dissociative group (indicated by Z of the general formula). Thus, the phot-ion-dissociation reaction is selectively induced according to wavelength of irradiating optical ray. Therefore, different triphenylmetane compounds are selectively developed according to wavelength of irradiating optical ray.

Further, as shown in Fig. 12, the color density can be regulated by changing the irradiating time interval of optical ray having wavelength of 340 nm and 300 nm. For example, from the curve 3 of Fig. 12 showing relation between the irradiating time interval and the color density, it is understood that when the irradiating time interval of the 340 nm optical ray is 1 sec the color density is 0.095, and when the irradiating time interval is 2 sec the color density is 0.385. Further, from the curve 4 of Fig. 12, it is understood that when the irradiating time interval of the 300 nm optical ray is 1 sec the color density is 0.140, and when the irradiating time interval is 2 sec the color density is 0.580. Therefore, the color density can be controlled according to the irradiating time interval.

As described above, at least one kind of triphenylmethane compound is directly impregnated in a substrate as the photo-sensitive color former exhibiting photochromism. The substrate is irradiated by optical ray to dissociate the photo-sensitive color former to record monocolor or multicolor image.

Further, the photo-sensitive color former has sensitivity to different wavelengths such that the color former can be selectively developed according to the wavelength of the irradiating optical ray. For this, multicolor forming can be effected according to the wavelength of the irradiating optical ray.

Moreover, by controlling the irradiating time interval, the color density can be regulated to thereby record monocolor or multicolor continuously gradated image of high resolution and high quality.

Still moreover, the substrate is directly impregnated with at least one kind of triphenylmethane compound as the photo-sensitive color former such that the recording paper has a simple mono-layer structure -- not complicated multi-layer structure, thereby facilitating the mass production.

### Example 1

There was utilized, as the photo-sensitive color former, malachite green leuco cyanide represented by the following formula: The 18.0 weight part of this malachite green leuco cyanide was dissolved into 500 ml of chloroform. A 33.0 g/cm² of free sheet of paper having the dimension of 15 cm x 21 cm was dipped into the solution. The impregnation and drying were effected to produce the photochromic recording paper.

The thus obtained photochromic recording paper was irradiated with optical ray having 2 cm of spot diameter by xenon lamp of 300W to effect photo-sensitive color forming. The light absorption spectrum of the formed color image is shown in Fig. 1. Further, the relation between the irradiating time and the color density is shown in Fig. 2 in which the color density was measured while changing the irradiating time interval. As seen from Fig. 2, when the irradiating time was 1 sec, the color density was 0.095. When the irradiating time was 2 sec, the color density was 0.385. consequently, by changing the irradiating time, the color density was continuously changed to achieve the continuous gradation expression of image.

### Example 2

There was utilized, as the photo-sensitive color former, brilliant green leuco cyanide represented by the following formula: The 18.0 weight part of this brilliant green leuco cyanide was dissolved into 500 ml of chloroform. A 33.0 g/cm² of free sheet of paper having the dimension of 15 cm x 21 cm was dipped into the solution. The impregnation and drying were effected to produce the photochromic recording paper.

The thus obtained photochromic recording paper was irradiated with optical ray having 2 cm of spot diameter by xenon lamp of 300W to effect photo-sensitive color forming. The light absorption spectrum of the formed color image is shown in Fig. 3. Further, the relation between the irradiating time and the color density is shown in Fig. 4 in which the color density was measured while changing the irradiating time interval. As seen from Fig. 4, when the irradiating time was 1 sec, the color density was 0.090. When the irradiating time was 2 sec, the color density was 0.260. Consequently, by changing the irradiating time, the color density was continuously changed to achieve the continuous gradation expression of image.

### Example 3

There was utilized, as the photo-sensitive color former, crystal violet leuco cyanide represented by the following formula: The 18.0 weight part of this crystal violet leuco cyanide was dissolved into 500 ml of chloroform. A 33.0 g/cm² of free sheet of paper having the dimension or 15 cm x 11 cm was dipped into the solution. The impregnation and drying were effected to produce the photochromic recording paper.

The thus obtained photochromic recording paper was irradiated with optical ray having 2 cm of spot diameter by xenon lamp of 300W to effect photo-sensitive color forming. The light absorption spectrum of the formed color image is shown in Fig. 5. Further, the relation between the irradiating time and the color density is shown in Fig. 6 in which the color density was measured while changing the irradiating time interval. As seen from Fig. 6, when the irradiating time was 1 sec, the color density was 0.085. When the irradiating time was 2 sec, the color density was 0.360. Consequently, by changing the irradiating time, the color density was continuously changed to achieve the continuous gradation expression of image.

### Example 4

There was utilized, as the photo-sensitive color former, rosaniline leuco cyanide represented by the following formula: The 18.0 weight part of this rosaniline leuco cyanide was dissolved into 500 ml of acetone. A 33.0 g/cm² of free sheet of paper having the dimension of 15 cm x 21 cm was dipped into the solution. The impregnation and drying were effected to produce the photochromic recording paper.

The thus obtained photochromic recording paper was irradiated with optical ray having 2 cm of spot diameter by xenon lamp of 300W to effect photo-sensitive color forming. The light absorption spectrum of the formed color image is shown in Fig. 7. Further, the relation between the irradiating time and the color density is shown in Fig. 8 in which the color density was measured while changing the irradiating time interval. As seen from Fig. 8, when the irradiating time was 1 sec, the color density was 0.145. When the irradiating time was 2 sec, the color density was 0.580. consequently, by changing the irradiating time, the color density was continuously changed to achieve the continuous gradation expression of image.

### Example 5

There was utilized, as the photo-sensitive color former, pararosaniline leuco cyanide represented by the following formula: The 18.0 weight part of this pararosaniline leuco cyanide was dissolved into 500 ml of acetone. A 33.0 g/cm² of free sheet of paper having the dimension of 15 cm x 21 cm was dipped into the solution. The impregnation and drying were effected to produce the photochromic recording paper.

The thus obtained photochromic recording paper was irradiated with optical ray having 2 cm of spot diameter by xenon lamp of 300W to effect photo-sensitive color forming. The light absorption spectrum of the formed color image is shown in Fig. 9. Further, the relation between the irradiating time and the color density is shown in Fig. 10 in which the color density was measured while changing the irradiating time interval. As seen from Fig. 10, when the irradiating time was 1 sec, the color density was 0.100. when the irradiating time was 2 sec, the color density was 0.510. Consequently, by changing the irradiating time, the color density was continuously changed to achieve the continuous gradation expression of image.

### Example 6

The photo-sensitive color former was comprised of the following two triphenylmethane compounds: An 18.0 weight part of malachite green leuco cyanide and an 18.0 weight part of rosaniline leuco cyanide were dissolved into 1ℓ of chloroform. A 33.0 g/m² of free sheet shaped in 15 cm x 21 cm size was dipped into the thus prepared solution. The two triphenylmethane compounds were impregnated and dried to form the multicolor photochromic recording paper.

The thus obtained multicolor photochromic recording paper was irradiated with an optical ray of 340 nm and 300 nm having a spot diameter of 2 cm by a xenon lamp of 300W through an optical filter to photo-sensitively form color image. The light absorption spectrum of the thus obtained double color image is shown in Fig. 11, and the relation between the irradiating time interval and the color density is shown in Fig. 12. From the curve 3 of Fig. 12 showing the relation between the irradiating time interval of 340 nm ray and the color density, it was recognized that the color density was 0.095 when the irradiating time interval was 1 sec, and the color density was 0.485 when the irradiating time interval was 2 sec. Further, from the curve 4 of Fig. 12 showing the relation between the irradiating time interval of 300 nm ray and the color density, it was recognized that the color density was 0.140 when the irradiating time interval was 1 sec, and the color density was 0.580 when the irradiating time interval was 2 sec. By such operation, the color density was continuously gradated by changing the irradiating time interval. Consequently, multicolor image of continuous gradation was realized.

### Example 7

The photo-sensitive color former was comprised of the following two triphenylmethane compounds: An 18.0 weight part of malachite green leuco cyanide and an 18.0 weight part of pararosaniline leuco cyanide were dissolved into 1ℓ of chloroform. A 33.0 g/m² of free sheet shaped in 15 cm x 21 cm size was dipped into the thus prepared solution. The two triphenylmethane compounds were impregnated and dried to form the multicolor photochromic recording paper.

The thus obtained multicolor photochromic recording paper was irradiated with an optical ray of 340 nm and 300 nm having a spot diameter of 2 cm by a xenon lamp of 300W through an optical filter to photo-sensitively form color image. The light absorption spectrum of the thus obtained double color image is shown in Fig. 13, and the relation between the irradiating time interval and the color density is shown in Fig. 14. From the curve 7 of Fig. 14 showing the relation between the irradiating time interval of 340 nm ray and the color density, it was recognized that the color density was 0.095 when the irradiating time interval was 1 sec, and the color density was 0.485 when the irradiating time interval was 2 sec. Further, from the curve 8 of Fig. 14 showing the relation between the irradiating time interval of 300 nm ray and the color density, it was recognized that the color density was 0.127 when the irradiating time interval was 1 sec, and the color density was 0.622 when the irradiating time interval was 2 sec. By such operation, the color density was continuously gradated by changing the irradiating time interval. Consequently, multicolor image of continuous gradation was realized.

### Example 8

The photo-sensitive color former was comprised of the following two triphenylmethane compounds: An 18.0 weight part of brilliant green leuco cyanide and an 18.0 weight part of rosaniline leuco cyanide were dissolved into 1ℓ of chloroform. A 33.0 g/m² of free sheet shaped in 15 cm x 21 cm size was dipped into the thus prepared solution. The two triphenylmethane compounds were impregnated and dried to form the multicolor photochromic recording paper.

The thus obtained multicolor photochromic recording paper was irradiated with an optical ray of 340 nm and 300 nm having a spot diameter of 2 cm by a xenon lamp of 300W through an optical filter to photo-sensitively form color image. The light absorption spectrum of the thus obtained double color image is shown in Fig. 15, and the relation between the irradiating time interval and the color density is shown in Fig. 16. From the curve 11 of Fig. 16 showing the relation between the irradiating time interval of 340 nm ray and the color density, it was recognized that the color density was 0.090 when the irradiating time interval was 1 sec, and the color density was 0.460 when the irradiating time interval was 2 sec. Further, from the curve 12 of Fig. 16 showing the relation between the irradiating time interval of 300 nm ray and the color density, it was recognized that the color density was 0.119 when the irradiating time interval was 1 sec, and the color density was 0.554 when the irradiating time interval was 2 sec. By such operation, the color density was continuously gradated by changing the irradiating time interval. Consequently, multicolor image of continuous gradation was realized.

### Example 9

The photo-sensitive color former was comprised of the following two triphenylmethane compounds: An 18.0 weight part of brilliant green leuco cyanide and an 18.0 weight part of pararosaniiine leuco cyanide were dissolved into 1ℓ of chloroform. A 33.0 g/m² of free sheet shaped in 15 cm x 21 cm size was dipped into the thus prepared solution. The two triphenylmethane compounds were impregnated and dried to form the multicolor photochromic recording paper.

The thus obtained multicolor photochromic recording paper was irradiated with an optical ray of 340 nm and 300 nm having a spot diameter of 2 cm by a xenon lamp of 300W through an optical filter to photo-sensitively form color image. The light absorption spectrum of the thus obtained double color image is shown in Fig. 17, and the relation between the irradiating time interval and the color density is shown in Fig. 18. From the curve 15 of Fig. 18 showing the relation between the irradiating time interval of 340 nm ray and the color density, it was recognized that the color density was 0.090 when the irradiating time interval was 1 sec, and the color density was 0.460 when the irradiating time interval was 2 sec. Further, from the curve 16 of Fig. 18 showing the relation between the irradiating time interval of 300 nm ray and the color density, it was recognized that the color density was 0.130 when the irradiating time interval was 1 sec, and the color density was 0.632 when the irradiating time interval was 2 sec. By such operation, the color density was continuously gradated by changing the irradiating time interval. consequently, multicolor image of continuous gradation was realized.

## Claims

1. A photochromic recording medium comprising: a paper substrate; and photochromic material composed of triphenylmethane compound impregnated in the paper substrate and responsive to irradiation of optical ray effective to develop the photochromic material so as to effect recording of image on the paper substrate, the triphenylmethane compound having general composition represented by the following formula: where X₁, X₂ and X₃ denote: hydrogen atom, halogen atom, alkyl group, alkoxyl group, amino group including the type in which hydrogen atom is substituted by alkyl group, alkoxyl group, alkyl halide group, phenyl group or phenyl halide group, and nitro group,
Y₁ and Y₂ denote: hydrogen atom, halogen atom, alkyl group, alkoxyl group, and amino group including the type in which hydrogen atom is substituted by alkyl group, alkoxyl group, alkyl halide group, phenyl group or phenyl halide group,
and Z denotes: hydroxyl group, cyano group, alkoxyl group and halogen atom.

2. A photochromic recording medium according to claim 1; wherein the photochromic material is comprised of a plurality of different kinds of the triphenylmethane compounds responsive to different wavelengths of optical ray to form different color tones to affect recording of multicolor image.
